

G. W. CHIPLEY  
BRAKE SHOE.  
APPLICATION FILED AUG. 5, 1914.

1,136,936.

Patented Apr. 27, 1915.

Fig. 1.



Fig. 2.



Fig. 3.



WITNESSES

A. V. Haleh.  
George Cook.

INVENTOR

Gardiner W. Chipley  
BY George Cook  
ATTORNEY

# UNITED STATES PATENT OFFICE.

GARDINER W. CHIPLEY, OF LOS ANGELES, CALIFORNIA.

## Brake-Shoe.

1,136,936.

Specification of Letters Patent. Patented Apr. 27, 1915.

Application filed August 5, 1914. Serial No. 855,129.

To all whom it may concern:

Be it known that I, GARDINER W. CHIPLEY, a citizen of the United States, and a resident of Los Angeles, in the county of Los Angeles and State of California, have made and invented certain new and useful Improvements in Brake-Shoes, of which the following is a specification.

My invention relates to an improvement in brake shoes particularly adapted for use in connection with railroad and railway cars. Heretofore brake shoes to be employed in such service have usually been constructed of metal, such, for instance, as cast iron, cast steel, etc., but certain objections have been urged against the use of metal and for various reasons. In the first place, it is well known that in order to give to the shoe a high co-efficient of friction, the metal must be comparatively soft, but when made up entirely of such metal, the life of the shoe is necessarily a short one, as it rapidly wears or burns away, due to the excessive heat generated by its frictional contact with the tread of the wheel. If, however, the shoe be made of comparatively hard metal, in order to prolong the life thereof, it is apt to score, cut, or otherwise injure the tread of the wheel; furthermore, being brittle in its nature, is apt to crack or break while in service. To overcome these objections, it has been common in the art to give to the shoe a composite wearing face, that is, to construct the shoe partly of hard, and partly of soft, metal, by the use of inserts, the result being that the shoe becomes expensive to manufacture.

The object of my invention is to produce a shoe which will possess both frictional and lasting qualities, and at the same time be comparatively cheap to manufacture, and also light in weight, in order to materially decrease the cost of transportation or shipping the same from the foundries to the place of service.

With these and other ends in view, the invention consists of a brake shoe constructed of hydraulic cement, reinforced throughout the major portion thereof by metal, in order to prevent injury thereto, and to hold the sections together in the event that the shoe should become cracked or broken.

The invention further consists in certain

novel features of construction as will be hereinafter fully described and pointed out in the claims.

In the accompanying drawing, Figure 1 is a view in side-elevation of a brake shoe constructed in accordance with my invention. Fig. 2 is a plan view, partly in elevation, and partly in section, to illustrate the metal reinforcement contained in the body thereof. Fig. 3 is a sectional view taken on the line 3—3 of Fig. 2, and looking in the direction as indicated by the arrow.

Referring to the drawings, it will be seen that the shoe is of the usual configuration or type, the body 4 thereof being curved in its length to conform to the curvature of the wheel, and provided centrally with a lug 5 for its attachment to a brake head (not shown), this lug being preferably made of wrought metal, the lower ends 6 thereof being outwardly flanged or bent, and anchored in the body of the shoe. This lug is preferably entirely surrounded by the cement of which the body 4 is constructed, with the exception of its upper side, the wrought metal lug 5 thus reinforcing the cement which partially forms the attaching lug. The shoe, if desired, is also formed with the end stops 7 and guide lugs 8, as are usual in this type of shoe.

The body of the shoe, as above stated, is made of hydraulic cement, such, for instance, as Portland cement, either alone, or mixed with other constituents, the mixture which I prefer consisting of about one portion of cement to two portions of sand, although, of course I do not intend to in any wise limit my claim to these proportions or even these constituents, the gist of my invention residing in the use of cement, either alone, or mixed with other ingredients to form the body of the shoe. In the shoe is contained a metal reinforcement 9 preferably in the form of expanded metal, wire mesh, or the like, although, of course, it will be understood, without further illustration or description, that the metal reinforcement 100 may assume any form, shape or configuration, as desired. In the drawing I have illustrated the shoe as containing three layers of expanded metal, running lengthwise of the shoe, and through the upper layer of 105 which extend the lower ends of the attach-

ing lug 5, in order to assist in firmly anchoring the latter to the body of the shoe. In molding this shoe, it is desirable that the mixture shall be of such consistency that it will, with certainty, fill all portions of the mold, and completely fill the interstices of the metal mesh, a sufficient quantity being first poured into the mold, then a layer of expanded metal, or its equivalent, placed in the mold, the mixture then again poured into the mold, and then a reinforcement inserted, and so on until the mold is completely filled. It is also desirable that the mixture be allowed to stand for several weeks in order that it will firmly and completely "set", and the moisture entirely evaporated.

It will be understood that a shoe constructed as described is comparatively cheap to manufacture; that it is light in weight, strong and durable in use, and possesses un-

usual frictional qualities, as well as lasting qualities.

What I claim is:—

1. A brake shoe the major portion of 25 which is constructed of hydraulic cement.
2. A brake shoe constructed of reinforced hydraulic cement.
3. A brake shoe the body of which is constructed of cement and containing a metal 30 reinforcement.
4. A brake shoe made of cement and sand, and the body of which contains a plurality of layers of expanded metal.

Signed at Los Angeles, in the county of 35 Los Angeles and State of California, this 10th day of July A. D. 1914.

GARDINER W. CHIPLEY.

Witnesses:

J. T. BREWER,  
C. G. WALLACE.